

## UNITED STATES PATENT OFFICE.

HENRI LOUIS BARTHÉLEMY, OF VERCELLI, ITALY, ASSIGNOR TO RUTH ALDO COMPANY INC., OF NEW YORK, N. Y., A CORPORATION OF NEW YORK.

PROCESS OF SOFTENING FIBERS OF CELLULOSE ORIGIN WITH A VIEW TO FACILITATING THEIR ESTERIFICATION.

No Drawing. Application filed January 27, 1928, Serial No. 249,987, and in France December 29, 1927.

Ever since the acetylation of cellulose has been practised, it has been recognized as advantageous to operate on a cellulose which has been subjected to a certain modification, 5 instead of on cellulose in its customary form.

It may even be said that a commencement was made with acetylating the hydrocelluloses; but it is known that the hydrolyzation of cellulose is a degradation of that 10 substance, which degradation, whilst considerably facilitating esterification, furnishes, in general, products which, in most instances, exhibit inferior plastic and mechanical properties.

15 The various authors of the processes for the acetylation of cellulose have busied themselves in seeking other preliminary treatments, such as:—

1. A partial preliminary esterification, for 20 example according to the French Patent No. 573,739 of 23rd November, 1923, which prescribes the use of formic acid; also the French Patent No. 473,399 of 12th June, 1914, which prescribes a slight preliminary 25 nitration of the cotton.

2. A preliminary mercerization, see the French Patent No. 507,472, filed 16th December, 1919.

3. A controlled preliminary oxidation of 30 the cotton as proposed by the applicant himself in the United States Patent Application No. 209,167 filed on 28th July, 1927, for an "Improvement in processes for the esterification of cellulose."

35 4. Action of sulphuric acid alone; see United States Patent No. 1,546,679 of 14th May, 1919.

By quite a different order of ideas, it has 40 been proposed to treat the cotton by simply soaking it with 10-40% of acetic acid at a temperature below 30° C. The object of this treatment is merely to cause the fiber to swell in the dilute acetic acid formed by the humidity of the cotton (see French Patent No. 596,802 of 28th July, 1924).

45 It has also been proposed, with a similar object, to force a certain quantity of acetic acid through the previously compressed mass of cotton (see United States Patent No. 50 1,466,401 of 28th August, 1923). Finally, applicant himself, in the first part of his

United States patent application No. 209,161 filed on the 28th July, 1927, for a "Process for the homogeneous esterification of cellulose," proposed to cause the vapor of 55 concentrated glacial acetic acid to pass through the mass of previously dried fibers.

Applicant has ascertained—and this is the object of the present invention—that the softening of the cuticle or the outer skin and 60 the internal tissue or pith of the cotton fibers can be considerably intensified, and that the duration of the treatment can be reduced in consequence, by combining with the action of the vapors of acetic acid, the action of 65 a small quantity of a halogen element, such as chlorine or bromine, or one of their reciprocal combinations, such as bromine chloride, BrCl, 10 Aq., iodine trichloride, &c.

This preliminary treatment not only 70 enables the cotton fiber to be more effectually and rapidly penetrated by the acetylating agents (thereby correspondingly diminishing the "waste" found after acetylation) but the fiber sustains a supplementary bleaching 75 at the same time. Moreover, the presence of a residual halogen in the fiber enables a considerably smaller amount of sulphuric acid to be employed in the acetylation bath, when said acid is used as the catalyst.

The temperature at which this small 80 amount of halogen element should be allowed to act is an important factor in obtaining good results. The temperature should not exceed 65°, and should preferably lie between 20° and 40° C.

The invention may be carried out in the various ways now enumerated, though these are not to be regarded as restrictive.

1. By introducing the halogens, in the 90 form of gas or vapor, into the mass of dry cotton prior to the vaporization or atomization of the acetic acid.

2. By introducing the acetic vapors simultaneously with the introduction of the halogen vapors.

3. By introducing the acetic vapors in the first place, following by the introduction of the halogen vapors in the second place.

4. By vaporizing, atomizing or nebulizing 100 the mixture (in strictly determined proportions) of the halogen element, or elements,

and the glacial acetic acid. Chlorine combines only very slowly, if at all, with pure acetic acid out of contact with light and in the absence of chlorination catalysts such as sulphur or iodine, and it is therefore possible to prepare such solutions several days in advance and to keep them in a comparatively satisfactory condition.

The nebulizing of the glacial acetic acid can be effected by means of apparatus producing a fine and relatively stable mist. For this purpose, use may advantageously be made of the apparatus described in Ullmann's "Encyclopädie der technischen Chemie," vol. 4, page 283, lines 39 et seq.

Several examples of the treatment will now be given.

*Example 1.*

1000 kg. of boiled and bleached cotton are treated with a current of chlorine gas for 15 minutes, the temperature being maintained between 20° and 22°. At the end of that time the chlorine in excess is swept away by a current of dry air, after which an equal quantity of 99.4% acetic acid is vaporized through the mass. After leaving to rest for an hour, the temperature, which has risen to about 40-45°, is allowed to re-

cede. Esterification is then performed, preferably in the manner indicated in the United States patent application No. 209,161 or United States patent application filed this same day in the name of the same inventor, for "Improvement in the esterification of cellulose."

*Example 2.*

100 kg. of glacial acetic acid (98-99.5% strength) and 250 grms. of pure bromine are mixed in an earthenware vessel, said mixture being afterwards nebulized through 100 kg. of cotton which has previously been raised to a temperature of 42° C. The cotton should be dried beforehand, so as not to contain more than 1% of natural moisture.

After cooling down, the acetylation is effected by the known means, in presence, for example, of sulphuric acid.

*Example 3.*

100 kg. of glacial acetic acid are vaporized, by boiling, into 100 kg. of carded dry cotton which has been previously raised to a temperature of 50° C. After cooling down to 23-25°, a current of chlorine gas is passed through the mass in such a way as to fix 0.5% of chlorine, referred to the weight of the cotton. This operation is followed by acetylation in known manner.

I claim:

1. A process for softening cellulose fibers in order to facilitate their esterification, con-

sisting in subjecting the mass of fibers to the combined action of the vapors of glacial acetic acid and an intensifying agent selected from the halogen group of elements.

2. A process for softening cellulose fibers in order to facilitate their esterification, consisting in introducing into the mass of fibers both halogen vapor and acetic acid vapor.

3. A process for softening cellulose fibers in order to facilitate their esterification, consisting in first introducing halogen vapor into the mass of dry fibers and then vaporizing acetic acid through the mass.

4. A process for softening cellulose fibers in order to facilitate their esterification, consisting in subjecting the mass of fibers to the combined action of the vapors of glacial acetic acid and an intensifying agent selected from the halogen group of elements, the temperature at which the intensifying agent is allowed to act not exceeding 65° C.

5. A process for softening cellulose fibers in order to facilitate their esterification, consisting in introducing into the mass of fibers both halogen vapor and acetic acid vapor, the temperature at which the halogen vapor is allowed to act not exceeding 65° C.

6. A process for softening cellulose fibers in order to facilitate their esterification, consisting in first introducing halogen vapor into the mass of dry fibers and then vaporizing acetic acid through the mass, the temperature at which the halogen vapor is allowed to act not exceeding 65° C.

7. A process of softening cellulose fibers in order to facilitate their esterification, consisting in nebulizing through the mass of fibers, after drying said mass and raising its temperature to about 42° C., a mixture of glacial acetic acid and at least one of the halogen elements.

8. A process for softening cellulose fibers in order to facilitate their esterification, consisting in subjecting the mass of fibers to the combined action of the vapors of glacial acetic acid and at least one of the halogen elements, for the purpose of softening both the cuticle and the internal tissue jointly and also fixing in a homogeneous manner in the total mass of the fibers acetic acid vapors and gaseous halogen adapted to lessen the amount of the catalyst to be afterwards employed.

9. The process of softening cellulose fibers before esterification, consisting in subjecting them to the action of vaporized glacial acetic acid and a gaseous intensifying agent selected from the halogen group of elements, substantially as herein described.

10. The process of softening cellulose fibers before esterification, consisting in subjecting them to the action of vaporized glacial acetic acid and a gaseous intensifying agent pertaining to the halogen group of elements to soften both the cuticle and

the internal tissue jointly and to lessen the amount of the sulphuric acid required for the esterification of the mass.

11. A process for softening cellulose fibers in order to facilitate their esterification, consisting in subjecting the mass of fibers to the combined action of the vapors

of glacial acetic acid and chlorine to soften both the cuticle and the internal tissue jointly and to lessen the amount of the sulphuric acid required for the esterification of the mass. 10

In testimony whereof I affix my signature.

HENRI LOUIS BARTHÉLEMY.